

# United States Patent Office

3,334,120

Patented Aug. 1, 1967

1

3,334,120

## ORGANOSILOXANE COPOLYMERS

George W. Holbrook and Harry M. Schiefer, Midland, Mich., assignors to Dow Corning Corporation, Midland, Mich., a corporation of Michigan

No Drawing. Filed June 10, 1963, Ser. No. 286,491  
10 Claims. (Cl. 260—448.2)

This application is a continuation-in-part of applicants' abandoned application Ser. No. 281,032, filed May 16, 1963 entitled, "Siloxane Copolymers."

This invention relates to organosiloxane copolymers containing halophenylsiloxane units and fluoroalkylsiloxane units which copolymers are particularly useful as lubricants and hydraulic fluids.

With the commercial advent of hydrocarbon substituted organosiloxanes it soon became apparent that these materials, particularly the methylsiloxanes, had many of the desirable properties required for lubricants operating over a wide range of temperature. These properties were: excellent high temperature stability, extremely low freezing point and a relatively slight change in viscosity with temperature. However, the hydrocarbon substituted siloxanes suffer from one serious defect; namely, that they were not satisfactory lubricants for sliding steel on steel bearing surfaces. Since steel is the primary metal employed in machinery the use of hydrocarbon substituted siloxanes as lubricants has been severely restricted.

The first major improvement in siloxane lubricants came with the introduction of halophenylsiloxanes such as those described in U.S. Patent 2,599,984. It was found that by incorporating halophenylsiloxane units into hydrocarbon substituted siloxanes one could greatly improve the lubricating quality of siloxanes. However, the improvement was not sufficiently good to make these materials generally satisfactory for the lubrication of steel sliding surfaces.

An even greater advance came with the introduction of fluoroalkyl substituted siloxanes such as trifluoropropylmethylsiloxane. Homopolymers of these materials are excellent lubricants for sliding steel on steel bearing surfaces and in most respects they are equivalent to the best hydrocarbon oils. However, the fluoroalkylsiloxanes suffer from the serious disadvantages that they have a relatively steep temperature viscosity slope and are not useable as lubricants at temperatures below -40° F. or as an aircraft hydraulic fluid below 0° F. Thus, fluoroalkylsiloxane homopolymer fluids are not useable as lubricants in a wide variety of applications which require that the lubricant function at low temperatures. As a result, there is a great need for a material which has the desirable high temperature stability and lubricating qualities of the fluoroalkylsiloxanes while also possessing excellent low temperature stability so as to enable one to use the fluids at low temperatures.

Attempts have been made to obtain this result by copolymerizing the fluoroalkylsiloxanes with methylsiloxanes. These copolymers do indeed have low temperature properties in that they remain fluid at temperatures below -65° F. However, the lubricating qualities of such copolymers are poorer than the fluoroalkyl homopolymers. Consequently, such copolymers are not the answer to the problem posed in this invention.

Applicants have found most unexpectedly that copolymers containing both fluoroalkylsiloxane units and halophenylsiloxane units as defined below have lubricating properties approaching, or better than, those of the fluoroalkyl homopolymers but still will operate at extremely low temperatures. Thus, the fluids of this invention fill a long standing need in the silicone lubricating art.

2

This invention relates to copolymers having  
(1) units of the group



and  $\text{R}_3\text{SiO}_{1/2}$  on the ends of the molecules, the remaining units in said copolymer being substantially all  
(2) units of the group consisting of

(a)  $\text{R}'\text{SiO}$

and

(b)  $\text{D}_2 - \text{Si} - \text{C}_6\text{H}_4 - \text{SiO} - \text{D}_2$

the total units (2) being present in amount of at least 24 mol percent of the total copolymer and any units (b) being present in amount from 0 to 25 mol percent of the amount of units (a) and in the amount of 0 to 15 mol percent of the total copolymer,

(3)  $\text{C}_n\text{G}_{2n+1} - \text{R}''' - \text{Q} - \text{CH} - \text{CH}_2 - \text{SiO}$

units in amount of at least 5 mol percent of the total copolymer,

(4)  $\text{X}_a - \text{C}_6\text{H}_4 - \text{SiO}_{1/2}$  and  $\text{X}_a - \text{C}_6\text{H}_4 - \text{SiO} - \text{Me}$

units in amount such that the total number of units of the formula



in said copolymer is from 1 to 15 mol percent of the total copolymer, and

(5)  $\text{ZSiO}_{3/2}$  units in amount of from 0 to 10 inclusive mol percent, said units being interconnected through SiOSi linkages in which

40 R is of the group methyl, phenyl, and



radicals, Q is of the group hydrogen and  $\text{C}_n\text{F}_{2n+1}\text{CH}_2\text{CH}_2 -$ , n is an integer from 1 to 8 inclusive,

R' and D are each of the group methyl and phenyl radicals, at least one R' and D per silicon being on the average a methyl radical,

R''' is of the group phenyl and methyl radicals,

Z is of the group phenyl, methyl and



radicals,

55 X is of the group chlorine and bromine, a is an integer from 1 to 4 inclusive, and

b has a value from 0 to 2 inclusive.

As can be seen, the copolymers of this invention are basically three or four component copolymers in which the first component is a triorganosilyl unit which serves as an endblocker. It should be understood that some of the molecular ends may contain hydroxyl groups or other extraneous groups but that essentially all the ends of the molecules are blocked with aforesaid groups (1). Thus, (1) can be any triorganosiloxy group in which the substituents on the silicon are methyl, phenyl or any of the defined fluoroalkyl groups such as trifluoropropyl, pentafluorobutyl,



It should be understood that any combination of these groups can be attached to the silicon of the triorganosiloxy group (1). In addition (1) can be any suit of the formula



Thus, specific examples of triorganosiloxy groups are trimethylsiloxy, triphenylsiloxy, phenyldimethylsiloxy, tribromophenyldimethylsiloxy, tetrachlorophenyldimethylsiloxy, monobromophenyldimethylsiloxy, trifluoropropylmethylsiloxy, bistrifluoropropylmethylsiloxy and



dimethylsiloxy.

The substituents (2) can be entirely dihydrocarbon-siloxy groups (a) in which the substituents are phenyl and methyl radicals or (2) can be made up of up to 25 mol percent based on the amount of (a) of (b) silphenylene units of the formula



in which D is phenyl or methyl. The total amount of silphenylene units, however, should not exceed 15 mol percent of the total copolymer. In all cases there should be an average of at least one methyl group per silicon atom in the total number of (2) units. Thus, (2) can be made up entirely of dimethylsiloxy units or of phenylmethylsiloxy units or any combination of these or (2) can be made up of combinations of dimethylsiloxy units and diphenylsiloxy units,



units or (2) can be a combination of phenylmethylsiloxy units with



units.

The fluoroalkylsiloxane units (3) are basically those which the fluoroalkyl radicals are of the formula  $\text{C}_n\text{F}_{2n+1}\text{CH}_2\text{CH}_2 -$  and telomers thereof of the formula



Specific examples of siloxane units (3) are trifluoropropylmethylsiloxane units, trifluoropropylphenylsiloxane units, heptafluoropentylmethylsiloxane units,  $\text{C}_8\text{F}_{17}\text{CH}_2\text{CH}_2\text{CH}_2$  methylsiloxane units,



and



It should be understood that the copolymers can contain any combination of these fluoroalkylsiloxane units. Thus, for example, the copolymer can contain both trifluoropropylmethylsiloxane units and pentafluorobutylmethylsiloxane units or the copolymer can contain both trifluoropropylmethylsiloxane units and trifluoropropylphenylsiloxane units.

One of the essential ingredients of the instant copolymers are the halophenylsiloxy groups. These must be

present in amount from 1 to 15 mol percent of the total copolymer. These groups can be of three types, namely,



and



10 The latter type of unit is also an endblocking unit (1) and if such units are present in amount to give a total of at least one mol percent halophenylsiloxy units in the copolymers, no additional halophenyl units are needed.

15 However, if desired a combination of any two or all three types of halophenyl units can be present in the copolymer. Thus, the halophenyl units can be located solely on the ends of the molecules or they can be located along the molecular chain of the copolymer or they can be 20 located in both positions in any particular copolymer.

Specific examples of operative halophenylsiloxy units, in addition to those shown under (1) above, are chlorophenylsiloxy units, dibromophenylmethylsiloxy units, tetrachlorophenylmethylsiloxy units, chlorodibromophenylsiloxy units, and tetrabromophenylsiloxy units.

The copolymers of this invention can also contain an optional ingredient (5) which is either monomethylsiloxane units, monophenylsiloxane units, or any



unit where Q and n are as defined above or any combination of these three types of units. Thus (5) can be  $\text{CF}_3\text{CH}_2\text{CH}_2\text{SiO}_{3/2}$ ,  $\text{C}_8\text{F}_{17}\text{CH}_2\text{CH}_2\text{SiO}_{3/2}$ ,



or



In any event, siloxane units (5) should not exceed a total of 10 mol percent of the copolymer.

The copolymers of this invention are best prepared by 45 cohydrolyzing the corresponding chlorosilanes followed by equilibration of the cohydrolyzate with alkali metal hydroxide catalysts or catalysts comprising the alkali metal salts of silanols. During the equilibration it is often desirable to remove water as it is formed and to maintain 50 the equilibrating system in an anhydrous condition. This is particularly true where the halophenyl substituents contain more than two halogen atoms. Thus, it can be seen that the copolymers of this invention are prepared by conventional techniques for copolymerizing siloxanes.

55 When silphenylene units are to be incorporated into the copolymer it is best to add the corresponding diol of the formula



60 to the acid free hydrolyzate containing the remaining ingredients and to equilibrate the mixture with the alkali line catalysts supra.

The starting halosilanes and diols from which the copolymers of this invention are prepared are all well-known materials.

The molecular size of the copolymers of this invention is not critical since they are all excellent lubricants regardless of polymer size. However, in many applications it is preferred that the viscosity of the copolymer be in the range from 25 to 10,000 cs. at 77° F. The copolymers of this invention are particularly desirable for use as hydraulic fluids and for this use a particularly desirable form has a viscosity from 50 to 150 cs. at 77° F. It is obvious that the viscosity of the co-

polymer will be determined by the mol ratio of triorganosiloxo groups to the other siloxy groups. Thus, the viscosity can be varied at will by increasing or decreasing the mol percent of triorganosiloxo groups in the system.

The compositions shown in the following examples were tested for lubricity on the Shell four-ball wear testing machine. In this test, a  $\frac{1}{2}$  inch steel ball is rotated against three stationary  $\frac{1}{2}$  inch steel balls at a rate of 1,200 r.p.m. at a temperature of 167° F. under loads of 4, 10 or 40 kilograms for 2 hours. At the end of this time the length and width of the scar formed on each stationary ball is determined and the average of these six measurements is taken as the scar diameter and reported in millimeters. The smaller the scar diameter, the better the lubricant.

of the chlorosilane mixture, the product was heated for 15 min. and cooled. About one liter of toluene was added and the organic phase was separated and washed with sodium bicarbonate solution until the toluene solution was neutral.

5 g. of KOH was added and the toluene was removed by distillation. The residue was heated and stirred for 16 hours at 160 to 170° C. 10 g. of  $\text{Me}_3\text{SiCl}$  was then added to neutralize the alkali and the product was then filtered and heated to 270° C. at .25 mm. under a slow  $\text{N}_2$  purge and then heated to 275° C. at 2 mm. under a vigorous  $\text{N}_2$  purge. The residue was then heated on a steam bath for two hours for 5 g. of  $\text{Na}_2\text{CO}_3$  and then filtered.

10 15 The Shell 4-ball wear tests were run at 167° F.

TABLE I

| Run No. | Composition of copolymer in mol percent |                                                   |                         |                                                              | Viscosity in cs. |         |         |         | Scar Diameter in mm. |        |
|---------|-----------------------------------------|---------------------------------------------------|-------------------------|--------------------------------------------------------------|------------------|---------|---------|---------|----------------------|--------|
|         | $\text{Me}_3\text{SiO}_{1/2}$           | $\text{Cl}_2\text{C}_6\text{H}_5\text{SiO}_{3/2}$ | $\text{Me}_2\text{SiO}$ | $\text{Me}$<br>$\text{CF}_3\text{CH}_2\text{CH}_2\text{SiO}$ | 77° F.           | 122° F. | 210° F. | -65° F. | 4 kg.                | 40 kg. |
|         |                                         |                                                   |                         |                                                              |                  |         |         |         |                      |        |
| 1.      | 10                                      | 5.0                                               | 60.0                    | 25                                                           | 142.6            | 55.6    | 25.5    | 37,000  | 0.29                 | 0.93   |
| 2.      | 10                                      | 5.0                                               | 65.0                    | 20                                                           | 101.7            | 41.8    | 19.7    | 8,161   | 0.20                 | 0.88   |
| 3.      | 10                                      | 5.0                                               | 70.0                    | 15                                                           | 77.0             | 34.9    | 16.9    | 1,233   | 0.20                 | 0.81   |
| 4.      | 10                                      | 5.0                                               | 75.0                    | 10                                                           | 80.8             | 38.9    | 17.7    | 4,179   | 0.19                 | 0.85   |
| 5.      | 10                                      | 4.0                                               | 71.0                    | 15                                                           | 72.2             | 33.2    | 16.6    | 4,189   | 0.23                 | -----  |
| 6.      | 10                                      | 4.7                                               | 60.3                    | 25                                                           | 100.8            | 47.6    | 21.1    | 10,340  | 0.30                 | 1.02   |
| 7.      | 10                                      | 4.5                                               | 65.5                    | 20                                                           | 71.4             | 32.5    | 16.8    | 4,740   | 0.25                 | 0.85   |
| 8.      | 10                                      | 6.0                                               | 54.0                    | 30                                                           | 132.2            | 48.9    | 22.3    | 42,700  | 0.26                 | 0.97   |
| 9.      | 10                                      | 3.0                                               | 47.0                    | 40                                                           | 100.3            | 53.1    | 18.8    | 14,840  | 0.15                 | 0.99   |
| 10.     | 10                                      | 3.5                                               | 46.5                    | 40                                                           | 93.5             | 49.9    | 18.2    | 9,283   | 0.13                 | 1.05   |

The following examples are illustrative only and should not be construed as limiting the invention which is properly delineated in the appended claims. In the specification and claims the abbreviation Me is employed for the methyl radical.

#### Example 1

1000 g. of a copolymer of 6.2 mol percent dichlorophenylsiloxane, 75.3 mol percent dimethylsiloxane, 13.5 mol percent trimethylsiloxane and 5 mol percent phenylmethylsiloxane was mixed with 200 g. of



and 10 g. of KOH and the mixture was stirred and heated for 18 hours at 160 to 170° C. The resulting fluid was neutralized with  $\text{Me}_3\text{SiCl}$ , filtered and the volatiles were removed by heating to 255° C. at 1 mm. The resulting copolymer had the average composition: 5.6 mol percent dichlorophenyl  $\text{SiO}_{3/2}$ , 67.6 mol percent  $\text{Me}_2\text{SiO}$ , 12.2 mol percent  $\text{Me}_3\text{SiO}_{1/2}$ , 4.9 mol percent  $\text{C}_6\text{H}_5(\text{Me})\text{SiO}$  and 9.7 mol percent  $\text{CF}_3\text{CH}_2\text{CH}_2(\text{Me})\text{SiO}$ .

This copolymer had the following properties:

| Temperature, ° F.: | Viscosity, cs. |
|--------------------|----------------|
| -65                | 4,990          |
| 77                 | 82.5           |
| 122                | 49.1           |

(Pour point -70° F.)

The fluid was tested on the Shell 4-ball wear tester and gave a scar diameter of .16 mm. after 2 hours at 1200 r.p.m. at 167° F. under a load of 4 kg.

#### Example 2

A series of fluids were made and tested as shown in the table below. In each case a mixture of  $\text{Me}_3\text{SiCl}$ ,  $\text{Me}_2\text{SiCl}_2$ ,  $\text{Cl}_2\text{C}_6\text{H}_5\text{SiCl}_3$  and



in the ratios needed to give the compositions shown below, was added to 2850 g. of water. Following addition

35

#### Example 3

Employing the procedure of Example 2, a copolymer having the following composition was obtained.

|    |                                                     |              |
|----|-----------------------------------------------------|--------------|
| 40 | $\text{CF}_3\text{CH}_2\text{CH}_2\text{SiO}_{1/2}$ | Mol per cent |
|    | $\text{Cl}_2\text{C}_6\text{H}_5\text{SiO}_{3/2}$   | 10           |
|    | $\text{Me}_2\text{SiO}$                             | 5            |

and

|    |                                               |    |
|----|-----------------------------------------------|----|
| 45 | $\text{CF}_3\text{CH}_2\text{CH}_2\text{SiO}$ | 20 |
|----|-----------------------------------------------|----|

The copolymer was a fluid having good low temperature stability and excellent lubricity for steel on steel bearing surfaces.

50

#### Example 4

Employing the procedure of Example 2, a copolymer was obtained having the following composition.

|    |                                                   |              |
|----|---------------------------------------------------|--------------|
| 55 | $\text{Me}_3\text{SiO}_{1/2}$                     | Mol per cent |
|    | $\text{Me}_2\text{SiO}$                           | 10           |
|    | $\text{Br}_2\text{C}_6\text{H}_5\text{SiO}_{2/2}$ | 65           |

and

|    |                                               |    |
|----|-----------------------------------------------|----|
| 60 | $\text{CF}_3\text{CH}_2\text{CH}_2\text{SiO}$ | 20 |
|----|-----------------------------------------------|----|

The copolymer was a fluid having good low temperature properties and was an excellent lubricant for steel.

65

#### Example 5

Employing the procedure of Example 2, a copolymer was obtained having a viscosity of 70.1 cs. at 77° F. and having the composition

|    |                                                   |              |
|----|---------------------------------------------------|--------------|
| 70 | $\text{Cl}_2\text{C}_6\text{H}_5\text{SiO}_{3/2}$ | Mol per cent |
|    | $\text{Me}_2\text{SiO}$                           | 4.8          |
|    | $\text{Me}_3\text{SiO}_{1/2}$                     | 61.9         |
|    | $\text{C}_6\text{H}_5(\text{Me})\text{SiO}$       | 11.0         |

and

|    |                                                          |      |
|----|----------------------------------------------------------|------|
| 75 | $\text{CF}_3\text{CH}_2\text{CH}_2\text{CH}_2\text{SiO}$ | 18.3 |
|----|----------------------------------------------------------|------|

The copolymer gave a scar diameter of 1.10 mm. when tested at 40 kg. and at 167° F. on the Shell 4-ball wear tester.

*Example 6*

The following copolymers are obtained when the following halosilanes are cohydrolyzed as shown in Example 2, and the cohydrolyzate is azeotroped dry with toluene and then equilibrated with



5

10

**8**  
*Example 7*

One mole of  $\text{MeSiCl}_3$ , .5 mol of  $\text{Cl}_2\text{C}_6\text{H}_5\text{SiCl}_3$ , 5.5 mol of  $\text{Me}_2\text{SiCl}_2$  and 1.5 mol of



were mixed and added with stirring to 3000 g. of water. The hydrolyzate was separated, washed neutral with water and then 1.5 mol of



as a catalyst.

|   | Halosilanes                                                                                                           | Mol Percent | Copolymer                                                                                                                  | Mol Percent |
|---|-----------------------------------------------------------------------------------------------------------------------|-------------|----------------------------------------------------------------------------------------------------------------------------|-------------|
| 1 | $\begin{array}{c} \text{Cl} \text{---} \text{C}_6\text{H}_4 \text{---} \text{SiCl} \\   \\ \text{Me}_2 \end{array}$   | 3           | $\begin{array}{c} \text{Cl} \text{---} \text{C}_6\text{H}_4 \text{---} \text{SiO}_{1/2} \\   \\ \text{Me}_2 \end{array}$   | 3           |
|   | $\text{Cl}_4\text{C}_6\text{H}_5\text{SiCl}_3$                                                                        | 1           | $\text{Cl}_4\text{C}_6\text{H}_5\text{SiO}_{3/2}$                                                                          | 1           |
|   | $\text{Me}_2\text{SiCl}_2$                                                                                            | 20          | $\text{Me}_2\text{SiO}$                                                                                                    | 20          |
|   | $(\text{C}_6\text{H}_5)_2\text{SiCl}_2$                                                                               | 5           | $(\text{C}_6\text{H}_5)_2\text{SiO}$                                                                                       | 5           |
|   | $\begin{array}{c} \text{Me} \\   \\ \text{CF}_3\text{CH}_2\text{CH}_2\text{SiCl}_2 \end{array}$                       | 71          | $\begin{array}{c} \text{Me} \\   \\ \text{CF}_3\text{CH}_2\text{CH}_2\text{SiO} \end{array}$                               | 71          |
| 2 | $\begin{array}{c} \text{Me} \\   \\ (\text{C}_6\text{H}_5)_2\text{SiCl} \end{array}$                                  | .01         | $(\text{C}_6\text{H}_5)_2\text{SiO}_{1/2}$                                                                                 | .01         |
|   | $\begin{array}{c} \text{Me} \\   \\ \text{Cl} \text{---} \text{C}_6\text{H}_4 \text{---} \text{SiCl}_2 \end{array}$   | 7.00        | $\begin{array}{c} \text{Me} \\   \\ \text{Cl} \text{---} \text{C}_6\text{H}_4 \text{---} \text{SiO} \end{array}$           | 7.00        |
|   | $\text{Me}_2\text{SiCl}_2$                                                                                            | 82.99       | $\text{Me}_2\text{SiO}$                                                                                                    | 82.99       |
|   | $\begin{array}{c} \text{Me} \\   \\ \text{C}_8\text{F}_{17}\text{CH}_2\text{CH}_2\text{SiCl}_2 \end{array}$           | 10.00       | $\begin{array}{c} \text{Me} \\   \\ \text{C}_8\text{F}_{17}\text{CH}_2\text{CH}_2\text{SiO} \end{array}$                   | 10.00       |
| 3 | $\text{Me}_3\text{SiCl}$                                                                                              | 30.0        | $\text{Me}_3\text{SiO}_{1/2}$                                                                                              | 30.0        |
|   | $\begin{array}{c} \text{Cl}_2 \text{---} \text{C}_6\text{H}_4 \text{---} \text{SiCl}_3 \end{array}$                   | 5.0         | $\begin{array}{c} \text{Cl}_2 \text{---} \text{C}_6\text{H}_4 \text{---} \text{SiO}_{3/2} \end{array}$                     | 5.0         |
|   | $\text{Me}_2\text{SiCl}_2$                                                                                            | 45.0        | $\text{Me}_2\text{SiO}$                                                                                                    | 45.0        |
|   | $\begin{array}{c} \text{C}_6\text{H}_5 \\   \\ \text{CF}_3\text{CH}_2\text{CH}_2\text{SiCl}_2 \end{array}$            | 5.0         | $\begin{array}{c} \text{C}_6\text{H}_5 \\   \\ \text{CF}_3\text{CH}_2\text{CH}_2\text{SiO} \end{array}$                    | 5.0         |
|   | $\begin{array}{c} \text{Me} \\   \\ \text{CF}_3\text{CH}_2\text{CH}_2\text{SiCl}_2 \end{array}$                       | 10.0        | $\begin{array}{c} \text{Me} \\   \\ \text{CF}_3\text{CH}_2\text{CH}_2\text{SiO} \end{array}$                               | 10.0        |
|   | $\text{MeSiCl}_3$                                                                                                     | 5.0         | $\text{MeSiO}_{3/2}$                                                                                                       | 5.0         |
| 4 | $\text{Me}_3\text{SiCl}$                                                                                              | 10          | $\text{Me}_3\text{SiO}_{1/2}$                                                                                              | 10          |
|   | $\begin{array}{c} \text{Cl}_2 \text{---} \text{C}_6\text{H}_4 \text{---} \text{SiCl}_3 \end{array}$                   | 4           | $\begin{array}{c} \text{Cl}_2 \text{---} \text{C}_6\text{H}_4 \text{---} \text{SiO}_{3/2} \end{array}$                     | 4           |
|   | $\text{Me}_2\text{SiCl}_2$                                                                                            | 55          | $\text{Me}_2\text{SiO}$                                                                                                    | 55          |
|   | $\begin{array}{c} \text{Me} \\   \\ \text{CF}_3\text{CH}_2\text{CH}_2\text{SiCl} \end{array}$                         | 30          | $\begin{array}{c} \text{Me} \\   \\ \text{CF}_3\text{CH}_2\text{CH}_2\text{SiO} \end{array}$                               | 30          |
|   | $\text{C}_8\text{H}_5\text{SiCl}_3$                                                                                   | 1           | $\text{C}_8\text{H}_5\text{SiO}_{3/2}$                                                                                     | 1           |
| 5 | $\begin{array}{c} \text{Cl}_2 \text{---} \text{C}_6\text{H}_4 \text{---} \text{SiCl} \\   \\ \text{Me}_2 \end{array}$ | 10          | $\begin{array}{c} \text{Cl}_2 \text{---} \text{C}_6\text{H}_4 \text{---} \text{SiO}_{1/2} \\   \\ \text{Me}_2 \end{array}$ | 10          |
|   | $\text{Me}_2\text{SiCl}_2$                                                                                            | 55          | $\text{Me}_2\text{SiO}$                                                                                                    | 55          |
|   | $\begin{array}{c} \text{Me} \\   \\ \text{CF}_3\text{CH}_2\text{CH}_2\text{SiCl}_2 \end{array}$                       | 34          | $\begin{array}{c} \text{Me} \\   \\ \text{CF}_3\text{CH}_2\text{CH}_2\text{SiO} \end{array}$                               | 34          |
|   | $\text{CF}_3\text{CH}_2\text{CH}_2\text{SiO}_{3/2}$                                                                   | 1           | $\text{CF}_3\text{CH}_2\text{CH}_2\text{SiO}_{3/2}$                                                                        | 1           |
| 6 | $\begin{array}{c} \text{Br}_2 \text{---} \text{C}_6\text{H}_4 \text{---} \text{SiCl} \\   \\ \text{Me}_2 \end{array}$ | 10          | $\begin{array}{c} \text{Br}_2 \text{---} \text{C}_6\text{H}_4 \text{---} \text{SiO}_{1/2} \\   \\ \text{Me}_2 \end{array}$ | 10          |
|   | $\text{Me}_2\text{SiCl}_2$                                                                                            | 70          | $\text{Me}_2\text{SiO}$                                                                                                    | 70          |
|   | $\begin{array}{c} \text{Me} \\   \\ \text{C}_7\text{F}_{15}\text{CH}_2\text{CH}_2\text{SiCl}_2 \end{array}$           | 20          | $\begin{array}{c} \text{Me} \\   \\ \text{C}_7\text{F}_{15}\text{CH}_2\text{CH}_2\text{SiO} \end{array}$                   | 20          |

500 ml. of toluene and 10 g. of KOH were added and mixture was heated and stirred as the toluene was distilled. When the mixture was toluene-free the copolymer was heated and stirred for 16 hours at 160 to 170° C. The fluid was cooled and neutralized with  $\text{Me}_3\text{SiCl}$ , filtered and stripped to 290° C. at 1.5 mm. The resulting fluid copolymer had the composition 10 mol percent  $\text{Me}_3\text{SiO}_{1/2}$ , 5 mol percent



10

55 mol percent  $\text{Me}_2\text{SiO}$ , 15 mol percent



and 15 mol percent



It gave a scar diameter of .333 mm. when tested on the 20 Shell 4-ball wear tester at 167° F. for 2 hours at 10 kg.

That which is claimed is:

1. As a lubricant a copolymer having  
(1) units of the group consisting of



25

and  $\text{R}_3\text{SiO}_{1/2}$  on the ends of the molecules, the remaining units in said copolymer being substantially 30 all

- (2) units of the group consisting of  
(a)  $\text{R}'_2\text{SiO}$  and



35

the total units (2) being present in amount of at least 24 mol percent of the total copolymer and any units (b) being present in amount of from 0 to 25 mol percent of the amount of units (a), and from 0 to 15 mol percent of the total copolymer,

(3)



45

units in amount of at least 5 mol percent of the total copolymer,

(4)



50

units in amount such that the total number of units of the formula



55

in said copolymer is from 1 to 15 mol percent of the total copolymer and

- (5)  $\text{ZSiO}_{3/2}$  units in amount of from 0 to 10 inclusive mol percent of the total copolymer, said units being interconnected through  $\text{SiOSi}$  linkages, in which

R is selected from the group phenyl, methyl and



65

radicals,

Q is selected from the group consisting of hydrogen and  $\text{C}_n\text{F}_{2n+1}\text{CH}_2\text{CH}_2-$ ,

n is an integer from 1 to 8 inclusive,

R' and D are each independently selected from the group consisting of phenyl and methyl radicals, at least one R' and D group per silicon being on the average a methyl radical,

75

$\text{R}'''$  is selected from the group consisting of methyl and phenyl radicals,  
Z is selected from the group consisting of phenyl, methyl and



radicals,

X is selected from the group consisting of chlorine and bromine,

a is an integer from 1 to 4 inclusive, and  
b has a value from 0 to 2 inclusive.

2. As a lubricant a copolymer in accordance with claim 1 having a viscosity of 50 to 10,000 cs. at 77° F.

3. As a lubricant a copolymer in accordance with claim 1 having a viscosity of from 50 to 150 cs. at 77° F.

4. As a lubricant a copolymer having

(1) trimethylsiloxy units on the ends of the molecules, the remaining units in said copolymer being substantially all

(2) dimethylsiloxy units in amount of at least 24 mol percent,

(3) 3,3,3-trifluoropropylmethylsiloxy units in amount of at least 5 mol percent and

(4) dichlorophenylsiloxy units in amount of from 1 to 15 mol percent.

5. As a lubricant a composition in accordance with claim 4 having a viscosity of from 25 to 10,000 cs. at 77° F.

6. As a lubricant a composition in accordance with claim 4 having a viscosity of from 50 to 150 cs. at 77° F.

7. As a lubricant a copolymer having

(1) trimethylsiloxy units on the ends of the molecules, the remaining units in said copolymer being substantially all

(2) dimethylsiloxy units in amount of at least 24 mol percent of the total copolymer,

(3)



units in amount of not more than 25 mol percent of the amount of (2) and not more than 15 mol percent of the total copolymer,

(4) 3,3,3-trifluoropropylmethylsiloxy units in amount of at least 5 mol percent of the total copolymer and

(5) dichlorophenylsiloxy units in amount of from 1 to 15 mol percent based on the total copolymer.

8. A method of lubricating moving metallic parts which comprises maintaining therebetween a copolymer having

- (1) units of the group consisting of



and  $\text{R}_3\text{SiO}_{1/2}$  on the ends of the molecules, the remaining units in said copolymer being substantially all

- (2) units of the group consisting of

(a)  $\text{R}'_2\text{SiO}$  and



the total units (2) being present in amount of at least 24 mol percent of the total copolymer and any units (b) being present in amount of from 0 to 25 mol percent of the amount of units (a), and from 0 to 15 mol percent of the total copolymer,



units in amount of at least 5 mol percent of the total copolymer,



## 11

units in amount such that the total number of units of the formula



in said copolymer is from 1 to 15 mol percent of the total copolymer and

(5) ZSiO<sub>3/2</sub> units in amount of from 0 to 10 inclusive mol percent of the total copolymer, said units being interconnected through SiOSi linkages, in which

R is selected from the group phenyl, methyl and



radicals,

Q is selected from the group consisting of hydrogen and C<sub>n</sub>F<sub>2n+1</sub>CH<sub>2</sub>CH<sub>2</sub>—,

n is an integer from 1 to 8 inclusive,

R' and D are each independently selected from the group consisting of phenyl and methyl radicals, at least one R' and D group per silicon being on the average a methyl radical,

R''' is selected from the group consisting of methyl and phenyl radicals,

Q is selected from the group consisting of phenyl, methyl and



radicals,

X is selected from the group consisting of chlorine and bromine,

a is an integer from 1 to 4 inclusive, and

b has a value from 0 to 2 inclusive.

9. A method of lubricating moving metallic parts which comprises maintaining therebetween a copolymer having

(1) trimethylsiloxy units on the ends of the molecules, the remaining units in said copolymer being substantially all

(2) dimethylsiloxy units in amount of at least 24 mol percent,

5

(3) trifluoropropylmethylsiloane units in amount of at least 5 mol percent and  
(4) dichlorophenylsiloane units in amount of from 1 to 15 mol percent.

10. A method of lubricating moving metallic parts which comprises maintaining therebetween a copolymer having

(1) trimethylsiloxy units on the ends of the molecules, the remaining units in said copolymer being substantially all

(2) dimethylsiloxy units in amount of at least 24 mol percent of the total copolymer,

(3)



units in amount of not more than 25 mol percent of the amount of (2) and not more than 15 mol percent of the total copolymer,

(4) trifluoropropylmethylsiloxy units in amount of at least 5 mol percent of the total copolymer and

(5) dichlorophenylsiloane units in amount of from 1 to 15 mol percent based on the total copolymer.

## References Cited

## UNITED STATES PATENTS

|           |         |                   |           |
|-----------|---------|-------------------|-----------|
| 2,599,984 | 6/1952  | Fletcher et al.   | 260—448.2 |
| 2,809,207 | 10/1957 | Gainer            | 260—448.2 |
| 2,894,969 | 7/1959  | Pierce            | 260—448.2 |
| 2,961,425 | 11/1960 | Pierce et al.     | 260—448.2 |
| 3,050,492 | 8/1962  | Polmanteer et al. | 260—448.2 |
| 3,061,545 | 10/1962 | Badger            | 252—49.6  |

## FOREIGN PATENTS

1,225,228 2/1960. France.

TOBIAS E. LEVOW, Primary Examiner.

SAMUEL H. BLECH, Examiner.

P. F. SHAVER, Assistant Examiner.